

Feb. 16, 1960

J. R. ROBERTS, ET AL  
METHOD OF PREVENTING EXCESSIVE SPRING-BACK  
OF DRY FELTED FIBER MATS

2,925,360

Filed Aug. 29, 1957

2 Sheets-Sheet 1



Figure 2



Figure 3



Figure 1

JAMES R. ROBERTS  
ERNEST H. COLLINS  
INVENTORS

*James G. Noller*  
ATTORNEY

Feb. 16, 1960

J. R. ROBERTS ET AL

2,925,360

METHOD OF PREVENTING EXCESSIVE SPRING-BACK  
OF DRY FELTED FIBER MATS

Filed Aug. 29, 1957

2 Sheets-Sheet 2



Figure 4

JAMES R. ROBERTS  
ERNEST H. COLLINS  
INVENTORS

*Leslie G. Noller*  
ATTORNEY

# United States Patent Office

2,925,360

Patented Feb. 16, 1960

1

2,925,360

## METHOD OF PREVENTING EXCESSIVE SPRING-BACK OF DRY FELTED FIBER MATS

James R. Roberts, Longview, and Ernest H. Collins, Kelso, Wash., assignors to Weyerhaeuser Company, a corporation of Washington

Application August 29, 1957, Serial No. 681,059

3 Claims. (Cl. 154—101)

This invention relates to the manufacture of felted mats from individualized ultimate wood fibers, and has particular reference to a method of preventing excessive "spring-back" of such mats after cold pressing and improvement of the handling properties of such cold-pressed mats in the further processing of the mats to consolidate them into densified wood fiber structures.

The manufacture of felted wood fiber structures may be carried out by two well-known general procedures used in effecting felts for the production of hardboard, softboard, insulation blankets and batts, and partially densified moldable boards. The two general procedures for effecting such mats involve the deposition of the wood fibers from a dilute liquid slurry, or the deposition of dry or moist fibers from a gaseous carrier onto a mat-forming surface. It is to the latter of these general procedures, known as the dry or air-felting process, that this invention is directed. Generally speaking, the dry or air felting method of effecting the fibrous mats involves impacting individualized ultimate wood fibers and opened-up bundles, or tracheids, of such ultimate fibers from a felting device onto a traveling foraminous surface by means of applying suction underneath the foraminous surface while the mat is being formed. The fibers are carried to the area of felting in a pneumatic tube under positive pressure, and passed through a perforated generally cylindrical surface into the mat-forming area. After the mat has been formed, it is carried by the foraminous belt into a cold-pressing area where the mat is consolidated to a predetermined density for further processing. In an alternative method of mat forming, the ultimate desired thickness of the mat may be built up in a series of felting stages wherein successive superimposed layers of the inter-felted ultimate wood fibers, which may be the same or different fibers, are formed in integral relation with each other. In either case, the ultimate wood fibers supplied to the felt by the air stream under positive pressure are derived from a defibering procedure such as is effected in an Asplund defibrator or other similar known means. Binders, such as thermosetting resins of the phenol-aldehyde type, and such other additives as may be desired are added to the fiber mass ahead of the felting area, generally in the defibering area, so that a uniform mixture of the binder and such additives will have been achieved prior to felting.

These air-laid felts or mats possess generally lower densities than wet-laid felts. A typical air-laid felt may have a density in the range of between 1-3 pounds per cubic foot. Further densification after the felt has been laid is necessary, therefore, in order to provide the mat with sufficient tensile strength so that it can be handled and used for such purposes as insulation blankets or moldable board, or so that it may be handled for further processing to a densified wood fiber structure such as hardboard. Such further densification is effected by cold-pressing the mat under suitable pressing means such as pressure rollers or pressure belts traveling around pairs

2

of rollers. This densification by cold pressing is effective for consolidating the mats for some purposes, particularly purposes where a low density end product is desired. Where a high density end product is desired, as in the case of densified wood fiber structures, such as hardboard, certain difficulties have been experienced in the handling and further processing of the mat which has been densified by cold-pressing or pre-pressing. The dry fibrous materials of which the mat is constituted have the bulk property of responding elastically to the release of an applied pressure and causing a "spring-back" to a thickness or density intermediate the compressed density under the applied pressure, and the density of the mass prior to compression. The mat then having the said intermediate density resulting from the "spring-back" tends to rupture by shearing and blowout when consolidated between platens in a hot press for densification to a thin hardboard. These effects are the result of the failure of a low density mat to provide sufficient tensile strength to withstand the disrupting stresses caused by the expulsion of the relatively large volume of air from within the mat upon the closing of the press platens. The rupture due to shearing can be controlled partially and the blowout reduced somewhat by interposing a wire screen or other rough surface between a press platen and one surface of the mat to supplement the tensile strength. Other means of correcting these faults of low density inter-felted mats have been suggested, such as the utilization of the bonding means by a pre-setting technique so as to provide a properly compressed density by interfiber adhesion. However, such methods preclude proper use of the resin binders during the final hot-pressing consolidation. Another suggestion involves subjecting at least one surface of the mat to heat and moisture while it is passing through the cold pressing area by surface application of steam-carried moisture. This procedure, proposed in U.S. Patent No. 2,635,301, issued April 21, 1953, to Dale L. Schubert et al., is subject to the disadvantages that the thus moistened fibers on the surface of the mat tend to adhere to the pressure rollers or belts under the pressure rollers and thus disrupt the surface structure of the air-laid mat, and also, that the non-surface fibers are free to produce an appreciable amount of "spring-back." Still another suggestion involves adjusting the moisture content of the mat to a high level to effect better consolidation on prepressing. This proposal has the disadvantage mentioned above of moistened surface fibers adhering to the pressure rollers and also of having greater expulsion of water and loss of water-solubles upon final consolidation. Furthermore, the increased moisture content requires a longer press cycle to insure proper drying and consolidation resulting in increased costs.

It has now been found that dry air-laid wood fiber felts may be made into dense, handleable and useful products which do not have the undesirable characteristics heretofore experienced, as outlined above. The novel method described below results in a densification of the air-laid wood fiber felts with a minimum of spring-back without the necessity of advancing the thermosetting of the bonding resins appreciably, and without adversely affecting the pressing, as in the case of addition of substantial amounts of moisture.

The new method by which these results are achieved consists essentially in drawing dry steam through the entire depth or thickness of a formed mat, having a predetermined moisture content, prior to cold pressing from a space above the mat, by application of suction or negative pressure to the underside of the mat through the foraminous belt carrying the mat to the cold-pressing area. The dry steam is drawn through the mat for such a period of time in its travel from the felt area to the

cold-pressing area and at such a negative pressure as to provide a quantity of the dry steam which will increase the temperature of the fibers comprising the mat to such a degree that the temperature of the mat at its center of cross-section, as the mat leaves the cold-pressing area, is at least 90° F., while the moisture content of the mat remains substantially the same.

A typical process sequence for the formation of densified wood fiber mats from ultimate wood fibers, in which this new method of treating the mat with dry steam for effecting an initial consolidation of the fibers prior to cold-pressing and reducing the amount of "spring-back" after cold-pressing, is that which is carried out in the manufacture of a plane-surfaced whole wood fiber mat. In such a process whole wood is reduced to chip form and is fed to a defibering apparatus such as the Asplund defibrator. In the defibrator the chips are subjected to an atmosphere of steam at a pressure in the range of between about 50-200 pounds per square inch and a corresponding temperature for saturated steam. The product of the defibrator, which consists predominantly of individualized ultimate fibers and opened up bundles or tracheids of such fibers, is discharged from the defibrator as a moist, fluffy mass. A bonding agent, such as a thermosetting resin of the phenol-aldehyde type, is added at the downstream side of the defibrator, and other additives, such as water repellents and flame-proofing agents, may be added in or ahead of the defibrator. The fibrous material containing the bonding agent and other additives may or may not be separated from the steam in which it is entrained as it emerges from the defibrator and is then dried to a moisture content of not more than 40%. It is then processed for the removal of any chips, ribbons, sticks, or large fiber bundles as may have been included with the ultimate fibers and small bundles of same upon leaving the defibrator. This fraction may be discarded or, preferably, is reprocessed prior to mixing with the acceptable fraction. The ultimate fiber fraction, which comprises the major portion of the mass, is then adjusted to a moisture content of between about 8 to 18%, and is suspended in superatmospheric pressure air.

At this point in the process reference may be made to the accompanying drawings wherein:

Figure 1 is a side view of a section of the apparatus included in the mat-felting and cold-pressing areas utilizing a single felter unit.

Figure 2 is a top view of the section shown in Figure 1.

Figure 3 is a section of the steam chamber shown in Figures 1 and 2 taken on the line 3-3 of Fig. 2.

Figure 4 is a side view of a section of the apparatus included in the mat-forming and cold-pressing areas utilizing a series of three felter units arranged in series relationship.

The suspension of the acceptable fiber fraction of the product of the defibrator, processed as above in air under positive pressure, is introduced into the pneumatic conduit 10 leading to the felter head 11, which is cylindrical in shape and provided with a revolving means 12 to aid in distributing the fibers uniformly, breaking up agglomerations, and forcing the fibers through the perforations in the felter head. At the felter head 11 the fibers are forced through the perforations or foramen principally by the pressure of the air carrying them into a space of atmospheric pressure 13 and onto a foraminous traveling collecting surface 14, which latter is generally a Fourdrinier type wire screen. On the opposite side of the traveling foraminous belt, which serves as the collecting surface for the mat, a predetermined and independently controlled reduced pressure is maintained through suction box 15 attached to the suction side of blower 16 through conduits 17, 18. The vehicular air passes through the foraminous collecting surface, whereas the fibers, due to the acceleration gained by passing through the pressure gradient from superatmospheric

pressure to subatmospheric pressure, are forcibly impacted together as an interfelted mass of fibers or mat 19 of substantially completely randomly oriented particles.

Immediately after the mat of fibers of the desired thickness leaves the felting area, it is carried by the foraminous traveling surface 14 between an overhead steam chamber 20 and a suction box 21 located on the underside of the foraminous traveling surface immediately under the steam chamber 20. The steam chamber is a 5-sided box or casket with its open side facing the top surface of the mat of fibers. It should be located as closely as possible to the surface of the mat and provision should be made for lowering and raising the steam chamber in order to accommodate mats of varying thickness. Alternatively, adjustable deckles can be supplied on the sides of the steam chamber so that adjustment to lower levels of the mat surface can be made. Dry steam is introduced under pressure through steam pipes 22 into the inner space of the steam chamber 20, which latter is at atmospheric pressure. In order to prevent any condensation of the steam on the sides of the steam chamber with resultant dripping onto the mat (which marks the finished board), the latter are heated by means of a heat conducting liquid medium which is maintained at a temperature substantially above the boiling point of water by introduction of steam under pressure to conduits 23. From the steam chamber, the steam, having approximately the temperature corresponding to the pressure of the steam supplied by steam pipes 22, is quickly drawn through the mat of fibers into suction box 21, from which it is evacuated by the negative pressure supplied by blower 16 in the arrangement shown in Fig. 1 where the same blower is used for evacuation of both the steam suction box and the felter suction box, or by blower 24, as shown in Fig. 4, where an independent blower is utilized for the evacuation of the steam suction box. The duration of the treatment of the mat by the steam being drawn through it is very short and the quantity of steam is adjusted to accommodate different thicknesses of mats. The amount of suction by which the steam is drawn through the mat is also adjusted so that in combination with the time of travel of the mat under the steam chamber the quantity of steam passing through the mat will increase the temperature of the mat at its cross-section center to approximately 90° F.-130° F. as measured at the cold-pressing area and at the same time will not appreciably change the adjusted moisture content of the mat. Dependent upon the above conditions and somewhat upon the thickness of the mat, the time of travel under the steamer should be in the range of from  $\frac{3}{4}$  second to 6 seconds. In the arrangement of Fig. 1, a balanced damper 25 is interposed between the exit from such suction box 21 and the suction side of blower 16 to provide control of the amount of reduced pressure applied to the steaming operation. Reduced pressures of from 3" to 15" of water are preferred at the speeds of travel mentioned above.

As the mat 19 passes under the steamer 20, its thickness is reduced by the action of the negative pressure drawing the steam through the mat structure, resulting in the removal of static charges from the fibers, thus effecting an initial consolidation of the interfelted wood fibers of the mat.

Immediately after leaving the steaming area the steamed mat passes through a cold-pressing area where it is compressed to a predetermined density of from about 10 to about 25 pounds per cubic foot. This may be accomplished by a single roller, coacting opposing rollers such as rollers 26 and 27 of Figure 1, or by moving converging pressure belts as shown at 28 in Fig. 4. These methods of cold pressing or pre-pressing are conventional. Upon emerging from the cold-pressing area, still carried by the foraminous belt upon which the mat was originally felted, the steam-treated and cold-pressed mat does not have any appreciable tendency to return to its thick-

ness or density prior to cold-pressing or prior to the steaming treatment, due to what is termed the "spring-back" of the fibers. Any "spring-back" which is experienced is limited to a return to a density of not less than 7 pounds. It is permanently densified to that density at which it has sufficient structural strength to be handled, stored, or transported. It is capable of being used for a number of purposes, or it may be placed into a platen press having relatively small openings, or so-called "day-light" provision. For further consolidation into densified hardboard the treated mat is cut into desired lengths and transported on cauls into a heated platen press. Due to the fact that the mat has retained the thickness which it had immediately after leaving the press area, thus enabling the use of smaller openings in the densifying platen press and a lower total press height, the latter may be closed quickly because of the reduced distance of travel between platens providing faster and more economical press cycles. Also, the use of a pre-densified mat of the invention provides for the manufacture of a thicker board with the same density or of a board of greater density for the same thickness from a given press opening than would be possible from the untreated or normal cold-pressed felts. The rush of air from the region within the mat does not split the mat or tend to blow portions of it out of the press, because of the greater density and structural strength of the mat as it enters the press.

In view of the high structural strength and greater density of the felted mats produced in accordance with this process, such mats, when used in the production of highly densified hardboard, may be placed into the platen hot-presses as self-sustaining units, rather than units which require a caul or screen for carrying and a caul or screen to prevent the air expelled from within the mat from disrupting the mat. Consequently, the boards may be pressed using only a single caul, a single screen, or neither, using in the latter case the press platens for both carrying and covering the mats.

The foregoing process may be further illustrated by reference to the following illustrative examples:

#### Example I

White fir Asplund fiber treated in the defibrator with 1% phenol-formaldehyde resin solids (Amres 6131, manufactured by American-Marietta Company), 2.5% petrolatum, and .5% aluminum sulphate, the percentages being based on the dry weight of the wood fiber, was suspended in air after adjusting the moisture content to 12%, and made into a flat felt having a thickness of about 3.25" in accordance with the above-described general procedure. A continuous mat of the fibers was made and this was cut into sections, some of which were merely cold-pressed under an unheated roller, and others submitted to the action of dry steam for a period of approximately 5 seconds by passing said dry steam from a heated steam chamber at atmospheric pressure through the felt into a suction box. These latter were then cold-pressed with an unheated roller under the same pressure as the unsteamed mats.

The mats or felts which were not treated with the dry steam retained a thickness of about 1.4" after the cold-pressing, and had a tensile strength of 8-16 ounces per square inch. The felts which were treated with the dry steam had a thickness of 1.0" after steaming, retained a thickness of .5" after cold pressing, and had a tensile strength of 176 ounces per square inch.

It was found that the mat which had not been treated with steam contained 12% moisture, while the mats which had been treated with steam contained 11.9% moisture. The temperature of the mats which were treated with dry steam was appreciably higher than that of the untreated mats, and was in the range of from 120-130° F.

Upon transporting the felted mats of this example to a hot press for further consolidation into a densified

structure, it was found that the felts which had not been treated with dry steam were difficult to handle and tended to "blow out" of the hot press and rupture when the press was closed. The mats which had been treated with steam were easily handled without damage and did not rupture or "blow out" as the press closed.

#### Example II

White fir Asplund fibers containing 2% Amres resin, 3% petrolatum, and .5% aluminum sulphate were prepared as in Example I and processed into matted felts in accordance with the general process described above. Some of the felts produced in accordance with this example were treated with dry steam caused to pass through the structure of the felted mat by suction applied in accordance with the general process described above for approximately 1.3 seconds prior to cold-pressing and raising the temperature in the range of 120-130° F. Others were treated similarly but the quantity of steam passing through the structure of the felted mat was reduced until the temperature of the mats prior to cold-pressing was in the range of 80-90° F. The felts which were treated in accordance with the process of this invention had an original thickness of 3.25", assumed a thickness of .87" after cold-pressing and were easily handled without damage and did not rupture or "blow out" as the press closed in further consolidation. It was found that the mats treated with a reduced quantity of steam and having a lower mat temperature assumed a thickness after cold-pressing of 1.25", were difficult to handle and tended to "blow out" of the hot press and rupture when the press was closed. The moisture content of the mats made in accordance with this example were in the range of about 11-16% before and after steaming.

#### Example III

White fir (*Abies concolor*) Asplund fiber consisting of individualized ultimate wood fibers and small bundles or tracheids of such fibers and containing 2.5% petrolatum, 1/2% aluminum sulphate, and 1% thermosetting phenol-formaldehyde resin solids (Amres 6130, manufactured by American-Marietta Company), based on the dry weight of the wood fiber and having an adjusted moisture content of about 12% was suspended in air at atmospheric pressure and passed continuously through a series of filters as shown in Fig. 4 at 10, following the general procedure described above. The thus suspended white fir wood fibers were continuously impacted onto a traveling screen of the Fourdrinier type into a felted mat consisting of superimposed integral layers of interfelted fibers having a thickness of 4". The thus prepared mat was carried on the traveling screen 14 to a cold-pressing area 28 during an elapsed time of approximately 8½ seconds, during which travel dry steam introduced at a reduced pressure of 20 pounds into the atmospheric pressure of the heated steam chamber 20 was drawn through the mat for a period of 1½ seconds by a negative pressure of 10" of water supplied through suction box 21 to the underside of the traveling screen 12. Upon entering the cold-pressing area the mat passed under a pressure belt 28 hydraulically loaded to press the mat to a thickness of ½" at the exit side. The mat was then cut to desired lineal sizes and passed into a hot-press where it was pressed to an ultimate thickness of ⅛" and a density of approximately 60 pounds per cubic foot.

The felted mat was reduced from its original thickness of 4" to about 2.25" under the steamer and increased in thickness after passing the cold-pressing area from a thickness of ½" under the exit prepress roller to a mat having a thickness of ⅛" and a density of 8.6 pounds per cubic foot. The temperature of the mat at its cross-section center, after leaving the prepress or cold-pressing area, was 120° F. The moisture content

of the mat before steaming was 12%, and after steaming was 12.5%.

This experiment was repeated while omitting the step of drawing the dry steam through the mat while applying negative pressure under the steamer. When so operating no reduction of the mat's thickness was effected ahead of the prepress or cold-press area. Upon passing the prepress area the mat increased in thickness from  $\frac{1}{2}$ " under the cold-press exit roller to a mat having a thickness of 2" and a density of 3.2 pounds per cubic foot. The temperature of the mat remained constant at ambient atmospheric temperature and the moisture content remained constant at 12%.

The mats which were treated by dry steam in accordance with this example were firm and easy to handle for cutting and feeding into the hot press. No "blow-out" of the fibers or shearing on the caul plate was experienced upon closing the press. The mats which were not treated with dry steam in accordance with this example were unstable and hard to handle for cutting and feeding into the hot press. Considerable "blow-out" and some shearing on the caul plates were experienced upon closing the press.

Having now described our invention and illustrated the best means of its operation, we claim as new:

1. In a process for the production of densified wood fiber structures which comprises dry felting a mixture of ultimate wood fibers and binder having an adjusted moisture content of from 8-18% onto a traveling foraminous surface to form a mat of fibers and binder, consolidating the mat by cold-pressing and further consolidating the cold-pressed mat to its ultimate thickness as a densified structure, the step of effecting an initial consolidation of the mat which comprises drawing high-temperature dry steam from a space of atmospheric pressure containing such high-temperature steam in admixture with air through the mat after the felting step and before the cold-pressing step by application of negative pressure to the underside of the mat through the foraminous surface, said dry steam being drawn through the mat for a predeter- 40

mined length of time depending upon the thickness of the mat and at a predetermined negative pressure depending upon the time selected such that the combination of time and negative pressure provides a quantity of dry steam to the mat which increases the temperature of the mat at its cross-section center after cold-pressing to at least 90° F. without appreciably increasing the moisture content of the mat.

2. In a process for the production of hardboard which comprises dry felting ultimate wood fibers and binder having an adjusted moisture content of about 12% onto a traveling foraminous surface to form a mat of the fibers and binder having a thickness of about 5", consolidating the mat by cold-pressing and further consolidating the cold-pressed mat to a flat hardboard structure having a thickness of  $\frac{1}{8}$ ", the step of effecting an initial consolidation of the mat which comprises drawing dry steam at the temperature of 135 pounds steam from a space at atmospheric pressure through the mat after the felting step and before the cold-pressing step by application of negative pressure to the underside of the mat through the foraminous surface, said dry steam being drawn through the mat for a period of 1½ seconds at a negative pressure of about 10" of water to produce a temperature at the cross-section center of the mat after cold-pressing of approximately 120° F. with no appreciable increase in the moisture content of the mat.

3. The process of claim 2 in which the wood fibers are white fir ultimate wood fibers and the binder is a thermosetting phenol-formaldehyde binder.

#### References Cited in the file of this patent

#### UNITED STATES PATENTS

|    |           |          |       |               |
|----|-----------|----------|-------|---------------|
| 35 | 2,208,511 | Ellis    | ----- | July 16, 1940 |
|    | 2,441,169 | Roman    | ----- | May 11, 1948  |
|    | 2,480,851 | Goss     | ----- | Sept. 6, 1949 |
|    | 2,464,301 | Francis  | ----- | Mar. 15, 1949 |
|    | 2,635,301 | Schubert | ----- | Apr. 21, 1953 |
|    | 2,655,458 | Collins  | ----- | Oct. 13, 1953 |
|    | 2,714,081 | Burgon   | ----- | July 26, 1955 |